

May 14, 1935.

C. M. HOWELL ET AL

2,001,023

CREPED PAPER

Filed Oct. 23, 1934



Fig. 1

Inventors  
Charles M. Howell  
James A. Clark  
By their Attorneys  
Howson & Howson

Patented May 14, 1935

2,001,023

# UNITED STATES PATENT OFFICE

2,001,023

## CREPED PAPER

Charles M. Howell, Springfield, and James d'A. Clark, Swarthmore, Pa., assignors to Scott Paper Company, Chester, Pa., a corporation of Pennsylvania

Application October 23, 1934, Serial No. 749,648

6 Claims. (Cl. 154—55)

This invention relates to the manufacture of creped paper products more particularly those used for personal purposes such as towels and toilet tissue.

5 One of the principal objects of the invention is to provide a soft absorbent paper which is at the same time particularly resistant to fracture in use.

10 Another object of the invention is to provide a paper which has a superior degree of softness and absorbency.

15 Other objects and advantages of the invention will be apparent from the description thereof set out below and from the claims.

20 As is well known in the manufacture of creped paper the web is formed from a fibrous suspension on a suitable forming cylinder or Fourdrinier machine, then picked off the forming wire by means of a felt, passed between rollers to express the surplus water and pressed against a heated drying cylinder and then creped thereoff by means of a scraper or doctor placed at an angle to and in contact with the face of the cylinder. The creped web is then dried, calendered and reeled up. During the creping step there are two distinct and separate methods employed for completing the manufacture depending on whether the tissue is of the lightest weight for example about 6 lbs. but usually below 10 pounds per 3000 square feet (24"×36"—500) which is used for facial tissue and the like, known technically as cellulose wadding or if the tissue is of a heavier basis weight between 10 and 15 pounds per 3000 square feet used for example for toilet paper and the like, and the heaviest tissue of over twenty-five pounds per 3000 square feet used for example for toweling and the like. In the case of the wadding or lightest weight tissue, it is made by pressing the moist web against a large diameter heated creping cylinder, and made at a speed not above that which allows the web to be virtually dry as it issues from the creping doctor when it is next wound up onto a reel for packaging operations. In the case of the tissues heavier than 10 pounds per 3000 square feet with a cylinder of a normal size and at commercial speeds for these tissues the web issues from the creping doctor not very much drier than when pressed against the drying cylinder because it will be readily appreciated

45 that as the point of contact with the cylinder the web contains at least 65 percent of moisture and is at a temperature usually not in excess of 100° F., it requires a substantial time in contact with the heated cylinder to raise the temperature to where evaporation can take place freely and to supply the necessary latent heat for evaporation. Consequently the time necessarily required to effect much drying of the heavier tissues has not been considered hitherto commercially available as modern large paper machines produce a web

of finished tissue for similar use at a rate of up to one thousand feet per minute.

5 It is known that the lightest weight issues which are virtually dried before creping, are specifically softer than the heavier weight tissues. By specific softness is meant the inherent softness of the paper after allowing for the effect of the greater substance. By experiment it was found that the specific softness of the tissue was proportional to (a) the degree of dryness at the creping doctor and (b) the extent which the tissue was dried in contact with the creping cylinder. It was further found that the function of the creping doctor is to disturb the cohesion between the fibres comprising the sheet and that the dryer the sheet at that point, the less the tendency for the fibre bonds to reform during the subsequent drying operation; furthermore an increased degree of drying on the cylinder causes a greater adhesion between the moist web and the surface of the cylinder which results in a greater resistance to the edge of the doctor blade and hence a more complete disruption of the fibrous structure. It is clear that this disruption of the bonds between the fibres not only leads to enhanced softness and absorbency but at the same time tends to destroy the specific strength of the sheet. Further experiments disclosed that the numerical product of the specific tensile strength and specific softness of a creped sheet of tissue prepared from different ingredients and in different ways is approximately a constant quantity. In addition to softness and absorbency another important fundamental requirement of tissues and towels is that they should possess a high degree of strength when in use, and as these experiments indicate, it is possible to obtain increased softness and absorbency only at the expense of specific strength.

10 15 20 25 30 35 40 45 50 55 60 A hitherto unknown fact was discovered; that the property of both towels and tissues which gives them strength in practice, is not tensile and bursting strength, as required for example in U. S. Government specifications for such products, but the property of stretch, which as far as we are aware, has not been there or elsewhere mentioned in this connection.

It is well known that any paper made from cellulose without the addition of a special water-proof binding agent, however strong it might be when dry, becomes extremely weak when moistened, more especially so with soft absorbent papers made from pulp which has been relatively lightly beaten or otherwise processed; for example all untreated paper towels have their dry tensile strength reduced to the order of only about ten ounces per inch of width when moistened and it will be appreciated that this is an insignificant amount compared to the relatively

large forces imposed by the knuckles upon a moist paper towel when used for drying of the hands. If in place of a towel, a piece of extremely thin rubber sheeting were used similarly to a towel to wipe the hands, even if the ultimate tensile strength of the sheeting were considerably less than that of a moist paper towel, it would not disintegrate during such use. Accordingly, as will be described, paper towels were then made having a stretch many times greater than hitherto deemed necessary for imparting softness and absorbency and it was discovered that the similarity with the rubber sheeting held good; and in addition to providing a towel with a marked resistance to disintegration during use, the properties of absorbency and softness were improved and a paper towel of markedly superior and hitherto unknown characteristics was obtained. Similarly toilet tissue was made with a high degree of stretch incorporated which proved much more resistant to fracture in practice than hitherto available.

It is clear that a considerable amount of stretch must be potentially available to such tissues before reasonable protection is provided other than from mere numbers of sheets used together, and it was found by experiment that a degree of potential stretch of much less than 15 percent yields a wholly inadequate protection to fracture when the tissue becomes moist. For the purposes of description and as setting out a form of mechanism which will operate in a very satisfactory and economical manner for producing a new soft paper product having a high potential stretch, the drawing illustrates a preferred form. In the figure, 1 indicates means of forming the paper web, shown as a Fourdrinier but it may take the form of a cylinder machine. 3 indicates the carrying felt and 2 the press section where excess water is expressed from the wet web in a well known way. 5 indicates the large heated receiving or creping cylinder onto which the web is pressed by means of the roll 4 and the wet web of paper is creped off by the doctor 6, the web being shown at 7, and the web is passed to a series of dryer rolls 8 from which the web goes through pair of calender rolls 9 and is finally reeled up at 10 where it is ready to be cut into the finished form.

With the diameter of the receiving dryer 5 about the same as that of the succeeding dryers 8, it was found in practice when retaining the same speed of production and attempting to substantially increase the amount of crepe given hitherto so as to be in accordance with the invention by improving the drying effect of the receiving dryer by raising its temperature, when the surface temperature of the receiving (or creping) drier approached that of boiling water, the web blistered while in contact with this dryer and uneven and unsatisfactory creping resulted. To overcome this difficulty without having to slow down considerably the whole paper machine and so add greatly to the costs of production, it was found necessary to substantially increase the size of the receiving drier 5 preferably to at least ten feet or say double that of the normal size remaining driers 8 so as to effect the necessary amount of drying at a temperature well below 212° F. at the same production speed as heretofore.

The dryer section 8 is driven at a peripheral speed lower than the receiving dryer 5, by about 10 percent or over, the maximum possible difference being governed by the ability of the

creped web to retain its crepe without being pulled out by its own weight and the tension imposed upon it, and its inherent strength to resist being pulled out. Its inherent strength is found to be governed by the dryness of the web after leaving the creping doctor, which should preferably be over 40 percent of its moist weight and also by its uncreped bulk, the bulkier the moist sheet, the more rigid it is and the better it resists being stretched while moist. The composition of the fibrous furnish is preferably selected so as to be inherently as bulky as possible. To further preserve the resulting crepe from being drawn out by the natural shrinkage of the web during drying, it is also desirable to gradually reduce the peripheral speed of the driers 8 towards the calenders, for example by slightly reducing their diameters successively or in successive groups.

By these means it is possible to produce a soft creped tissue of substantial substance and having a high degree of potential stretch. It will be understood that the potential stretch in a creped paper is made up of two components, first the stretch available through the imparted crepe and secondly the stretch available by the elasticity and length of the component fibres which amounts usually to about two to three percent but has been found in the case for example of certain pulps prepared by an alkaline process to give an elongation of as high as six percent before fracture. It is, therefore, possible to produce a creped tissue having a potential stretch of fifteen percent according to this invention with only nine percent of crepe being added.

For the purpose of definition the softness of the products is determined by the following method:

Cut parallel strips of paper in the machine and cross directions about one or two inches wide, insert the end of each strip in turn between a diametrically split horizontal spindle preferably about  $\frac{1}{2}$  inch in diameter, and adjust the overhanging length so that on rotating the spindle through 90 degrees the strip just flops over in the direction in which the spindle is being rotated as it is turned back and forth through 90 degrees. The overhanging lengths are then measured in inches for both the machine and cross directions. If the average overhanging length so found is  $l_m$  inches for the machine direction and  $l_c$  inches for the cross direction and the thickness of the strip is  $t$  thousandths of an inch, the average softness factor is calculated according to the following empirical formula:

$$\frac{10t}{l}$$

$l$  being either  $l_m$  or  $l_c$ , whichever is the greater. The test is carried out at 65% relative humidity and 70° F.

According to this method the values for the softness of commercial soft absorbent tissues range from 5.0 to over 10.0. A tissue having an average softness factor of over 5.0 is considered as soft.

For the purposes of definition the absorbency is determined by the following method:

Place one thickness of the tissue on a 4 mesh per inch wire screen and allow 0.1 millimeter of water to flow on to the tissue. The absorbency is the time in seconds from the contact of the water with the tissue until the drop is completely absorbed, as indicated by no further reflection

of light from it. The test is carried out at 65% relative humidity and 70° F.

If the drop is absorbed in less than 600 seconds (10 min.) the tissue is considered absorbent.

5 For the purposes of definition stretch means the percentage increase of the original length of a parallel strip of paper at the instant of rupture, when subjected to a slowly increasing tensile strain and is determined by well known means 10 at a temperature of 70° F. and a relative humidity of 65%.

The relative proportions of the stretch due to the added crepe and the inherent potential stretch of the fibrous structure may be determined 15 by reference to the stress strain diagram when drawn by a recording extensometer in a well known manner.

We are aware that various non-absorbent creped papers having a high degree of crepe or 20 stretch are known which are commonly used for decorative purposes and the like. The process for producing them is confined to a separate machine from that on which the paper is formed and dried, and is applied to the dried web of paper by 25 causing it to be stuck, by means of an added adhesive, to a creping cylinder and creping therefrom. As the adhesive used invariably detracts from its absorbency, as well as the fact that the fibrous structure of the paper is not disturbed as 30 it is when creping just after its formation and while still moist, the resulting product is neither soft nor absorbent according to the stated tests and no claims are directed towards such a product.

35 We are also aware that creped soft absorbent multiply tissues are known, such products being made from highly creped tissues, the web of which has been substantially fully dried on the creping cylinder before creping and in consequence of which the use of a relatively light substance, usually between six and ten pounds per 40 3000 square feet, is necessary and the separate sheets of wadding are combined into a multiply sheet of any desired composite substance by 45 superimposing a number of webs together with or without embossing. This type of construction gives an extremely soft product and also an absorbent one. Notwithstanding the fact that the stretch may be high, in some cases over 15 percent, the benefits of stretch as regards resistance 50 to disintegration do not materialize, because on account of the extreme thinness of the individual plies of the product and the fact that the plies cannot be made to be substantially integral with 55 each other and the extreme disruption of the fibrous structure occasioned by this process as soon as the product is moistened and gently rubbed, the top or individual layer breaks and rolls up, followed by the successive layers and 60 the whole product rapidly disintegrates. Consequently a product made from multiple thicknesses of sheets having individually a low basis weight, even though they may have a high degree of stretch, in practice proves more unsatisfactory as 65 regards disintegration than a single ply sheet possessing a low degree of stretch and of the same basis weight as the composite multiply sheet. We make no claim for such a multiply product unless the outer plies are composed of 70 tissue made in accordance with this invention when the objection cited becomes less valid.

In the appended claims, the term "towel" re-

fers to a paper article, the basis weight of such article being in excess of approximately twenty-five pounds per 3000 square feet. Further, the term "toilet tissue" refers to a paper article the basis weight of which exceeds approximately twelve pounds per 3000 square feet. Further, the term "cellulose wadding" refers to a paper article the basis weight of which is usually considerably less than that of toilet tissue and which has been substantially fully dried before creping 10 and is characterized by softness and flimsiness in the lighter weights and by the greater gloss or polish imparted to one surface by such drying, such gloss being especially noticeable in the heavier weights.

15 While this invention may be carried into effect with any paper machine adapted to the manufacture of tissue we are not aware that anyone has hitherto recognized the novel and unexpected results of imparting a high degree of crepe to 20 the heavier classes of tissues mentioned, nor are we aware of any paper towel or similar tissue except when made of cellulose wadding having a potential stretch in excess of ten percent. Indeed we have found that the great majority have 25 a much lesser percentage of stretch than ten available, being commonly between three and six percent. Furthermore, to produce such a product on a paper machine without the large receiving dryer which hitherto has not been used 30 for such tissues would severely limit the speed at which the products could be made and so make their production uneconomical.

35 It will be obvious that the invention may be applied to any paper products of which the desirable characteristics of softness and/or absorbency and the possession of a sufficient degree of stretch to give effective resistance to fracture or disintegration during use, for example paper for table napkins and the like, but for these particular 40 products high degree of absorbency is undesirable and sizing materials may accordingly be added to the paper.

We claim:

1. As a product of manufacture, a soft creped 45 multiply towel or toilet tissue paper whereof any ply is made of paper other than cellulose wadding, said product having a potential stretch of not less than fifteen percent.

2. As an article of manufacture, a single ply 50 paper towel having a potential stretch of not less than fifteen percent.

3. As an article of manufacture, a single ply sheet of soft toilet tissue paper other than cellulose wadding having a potential stretch of not 55 less than fifteen percent.

4. As a product of manufacture, a soft towel or toilet tissue paper other than cellulose wadding having an additional percentage of stretch incorporated therein by creping, the total potential 60 stretch of the product being not less than fifteen percent.

5. As an article of manufacture, a single ply, soft, absorbent paper towel having a potential stretch of not less than fifteen percent. 65

6. As an article of manufacture, a single ply, sheet of soft, absorbent toilet tissue paper other than cellulose wadding having a potential stretch of not less than fifteen percent.

70  
CHARLES M. HOWELL.  
JAMES D'A. CLARK.